

Sept. 14, 1948.

W. E. BLACKBURN

2,449,444

SELENIUM RECTIFIER

Filed Oct. 30, 1946



WITNESSES:

Edward Michaels  
Fre. C. Groome

INVENTOR

Wayne E. Blackburn.

BY

F. W. Taylor.  
ATTORNEY

## UNITED STATES PATENT OFFICE

2,449,444

## SELENIUM RECTIFIER

Wayne E. Blackburn, Wilkinsburg, Pa., assignor  
to Westinghouse Electric Corporation, East  
Pittsburgh, Pa., a corporation of Pennsylvania

Application October 30, 1946, Serial No. 706,758

4 Claims. (Cl. 175—366)

1

My invention relates to selenium rectifiers and, in particular, relates to an improved process for forming the blocking or barrier layer in such rectifiers. In accordance with the prior art, such barrier layers have been produced by exposing the free surface of the selenium to the vapors of certain materials while in vacuum, by chemically treating the selenium surface, and by depositing a film of organic material on the selenium surface by dipping in a suitable solution. The latter has, in general, been found to be the least expensive but difficulty arises because films of organic material are likely to decompose at the temperatures at which the rectifiers are heat-treated during subsequent steps of the manufacturing process. The barrier layer thereafter comprises some carbonaceous material of uncertain composition. Furthermore, if the rectifier is subjected to high temperatures during the subsequent operation, for example, by reason of the heat generated by losses within the rectifier itself, further decomposition of the organic material in the barrier layer occurs. Thus the maximum temperature, and hence load output of which the rectifier is capable in use is limited because such subsequent decomposition produces changes in the rectifier characteristics which cannot be tolerated.

One object of my present invention is to produce a barrier layer on the selenium of selenium rectifiers by a dipping process which produces an inorganic film on the free surface of the selenium.

Another object of my invention is to produce a selenium rectifier which is capable of operating at higher temperatures than were selenium rectifiers of the prior art.

Another object of my invention is to produce a selenium rectifier having more stable characteristics both electrically and chemically than did selenium rectifiers of the prior art.

Other objects of my invention will become apparent upon reading the following specification, taken in connection with the accompanying drawing, in which the single figure is a sectional view of a rectifier embodying the principles of my invention.

In the preferred embodiment of my invention, I produce the inorganic barrier layer by coating the selenium surface with a solution or suspension of a suitable inorganic salt in an organic liquid, and subsequently by driving off the organic material before completion of the rectifier.

The preferred method of making this rectifier is to first produce a coating of amorphous sele-

2

nium on a suitable base plate which may, for example, be sheet iron, sand blasted and nickel plated. Such a sheet iron base is selenium-coated by dipping the plate in a bath of the molten selenium and throwing off excess material through centrifugal force by rotating the plate after dipping. The base plate thus coated is then submerged in a hot solution or suspension of an inorganic salt in an organic solvent. I have found that salts which are most effective are those whose metals form stable oxides, sulfides or selenides.

As examples of the most suitable salts, I will mention uranium nitrate, zirconium nitrate, magnesium thiosulfate, gallium nitrate, zinc diethionate, potassium columbate, aluminum nitrate and cerous nitrate. The most desirable organic solvent to be employed is alcohol or acetone. The density of the salt in the solution has not been found by my experiments to date to be critical but may, for example, be that corresponding to saturation.

After withdrawal from the bath, the solvent soon evaporates leaving a coating of the dissolved salt on the surface of the selenium. A coating, which may be cadmium or a cadmium alloy well known in the art, may then be metal-sprayed onto the surface of this coating to form the counter-electrode. The unit thus produced is then submitted to a heat treatment comprising annealing for a period of about 120 minutes at a temperature of 200 degrees centigrade. This converts the amorphous selenium into crystalline selenium and at the same time causes the deposited film to produce the desired barrier layer. Thereafter the rectifier is, in accordance with a method well known in the art, subjected to "electrical forming" by impressing upon it an alternating voltage of 35 volts for a period of 60 minutes. The rectifier unit is then complete.

It is my present belief that the deposited inorganic salt undergoes chemical combination with the selenium on which it is deposited to form a selenide, or possibly combines with oxygen of the air to some extent. Since the exact reaction is uncertain, I will hereinafter arbitrarily refer to the combination above described as an oxy-salt of the metal.

Referring in detail to the drawing, a completed rectifier thus comprises a base plate 1 having on one surface a layer 2 of selenium, the free surface of the layer being covered with a barrier layer 3 resulting from the deposition of the above-mentioned inorganic salt. The free

face of the barrier layer 3 is coated with a counter-electrode 4 as above described.

I claim as my invention:

1. The method of producing a selenium rectifier which comprises the step of coating a free surface of selenium with a suspension of magnesium thiosulfate in a volatile organic solvent. 5
2. The method of producing a selenium rectifier which comprises the step of coating the free surface of selenium with a solution of magnesium thiosulfate in alcohol.
3. The method of producing a selenium rectifier which comprises the step of coating the free surface of selenium with a solution of magnesium thiosulfate in acetone. 10

15

4. A rectifier comprising a layer of selenium coated on one face with an oxy-salt of magnesium thiosulfate.

WAYNE E. BLACKBURN.

#### REFERENCES CITED

The following references are of record in the file of this patent:

#### UNITED STATES PATENTS

| Number    | Name            | Date           |
|-----------|-----------------|----------------|
| 2,137,316 | Van Geel et al. | Nov. 22, 1938  |
| 2,139,731 | De Boer et al.  | Dec. 13, 1938  |
| 2,173,249 | De Boer et al.  | Sept. 19, 1939 |